

## UNITED STATES PATENT OFFICE

FRITZ R. BISCHOFF, OF SANTA BARBARA, CALIFORNIA, ASSIGNEE TO HENRY J. ULLMANN, OF SANTA BARBARA, CALIFORNIA

## METALLIC COLLOID AND PROCESS OF PRODUCING THE SAME

No Drawing.

Application filed October 12, 1926. Serial No. 141,242.

This invention relates to metallic colloids and to a process of producing the same.

Metallic colloidal solutions, when prepared by electrical disintegration of metallic wires under water or other solvent in accordance with the well-known Bredig or Svedberg methods, are unstable if the metal of the colloid is readily oxidized. For example, aqueous colloidal solutions of the readily oxidizable metals like lead, zinc, iron, etc., are very unstable and decompose to oxides, hydroxides and carbonates through reaction with the water and air. The reaction products precipitate out of the colloidal solution. By preparing such metallic colloids in dilute gelatine or other protective dispersing agent, the life of the colloid is increased, for although oxidation occurs, the dispersing agent keeps the products in colloidal solution. Even, however, with the use of dilute gelatine as a dispersing agent, the resulting metallic colloid will stand up for only a short period of time, for example, a one-half per cent solution of lead will stand up for only about two days.

An object of the present invention is to provide an improved metallic colloid and process of producing the same which is adapted to resist oxidation for a considerable period of time and which is adapted to stand up or retain its colloidal form.

I have discovered that by the addition of aliphatic poly-hydroxy compounds to the solution of the dispersing agent at the time of preparation of the metallic colloid, the poly-hydroxy compounds will operate to inhibit oxidation of the metal in the colloid, with the result that the metallic colloid is stable and may be preserved for several weeks. As an example of aliphatic poly-hydroxy compounds which have been found suitable for use in the process, glucose, fructose, lactose and the like, when added to gelatine solutions used for preparing the colloid, greatly increase the stability of the metallic colloid against oxidation. Partial results also may be obtained by the use of saccharide, although the effect is much diminished. Apparently, the decomposition products of any aliphatic poly-hydroxy compound, whether

alcohols, aldehydes or ketones, which decomposition products are formed by the electric arc, exert inhibiting effects towards oxidation of metallic colloids. Glycerol, for example, is found to be effective poly-hydroxy alcohol.

The present invention also may be employed as a means for producing metals without the metals going into the colloidal state. For example, if a solution of mono or di saccharide is employed without the use of gelatine, a metallic colloid forms but does not stay dispersed, but sinks to the bottom of the receptacle. The saccharide in this case exerts its specific effect against oxidation but does not operate as a protective agent for dispersion.

The invention, together with various further objects and advantages thereof, will be understood from a description of a number of examples of metallic colloids and processes of producing them embodying the present invention. I have therefore hereafter set forth examples of the effect of certain saccharides and other poly-hydroxy alcohols upon the stability of a lead colloid, lead colloids being particularly readily oxidized and difficult to maintain in colloidal form.

In the production of a lead colloid, a dilute gelatine solution is first formed, for example by dissolving four grams of commercial gelatine in a liter of water. For the best results, the pH of the solution is adjusted to 7.5 (colorimetrically). To said solution is then added an aliphatic poly-hydroxy compound, for example, ten grams of either glucose, fructose, sucrose or glycerol. The solution is then subjected to a high frequency oscillatory arc between the electrodes of lead for a period of time, depending upon the concentration of the desired metallic colloid. The apparatus is preferably employed in the usual Bredig arrangement. The current is preferably adjusted so that the arc does not flame, but emits a yellow light. Black colloidal solutions of lead are formed. A suitable solution can be obtained in approximately five minutes time. Very dilute solutions of the colloid, such as contain less than .05 per cent lead, will remain stable due to the presence of a poly-

hydroxy compound for a period of time in excess of the time which the ordinary colloid will remain stable.

Without the employment of the inhibiting agent of the present invention, a lead colloidal solution containing slightly less than .05 per cent lead was found to be entirely decomposed in three hours, no trace of black color remaining, while similar metallic colloids produced by glucose, fructose, and glycerol solutions, respectively, were still entirely black except for a slight narrow white band at the top of the solution. A metallic colloid prepared from a sucrose solution will, at the end of three hours, be only half decomposed. Other poly-hydroxy compounds, such as lactose or mannose, act similarly to sucrose, although dextrin is even less efficient. Metallic colloids prepared by the use of dextrose, fructose and glycerol solutions containing less than .05 per cent lead are only half oxidized at the end of twelve hours, and several days are required before the black color disappears and the white product of oxidation is formed.

Another example of a process embodying the present invention or metallic colloid produced thereby is as follows: An aqueous solution containing .4 per cent gelatine and .5 per cent glucose is adjusted until its pH is between 7 and 8. If its pH is left between 5 and 7, lower yields will be obtained. The solution is then cooled such as by packing in ice, and subjected to a high frequency oscillatory arc, using lead electrodes for one and one-half hours. Preferably the solution is stirred continuously and maintained at a temperature below 30° C., throughout the process. The arc is preferably adjusted so that no flaming occurs. Optimum results are obtained when the gap between the electrodes is less than a millimeter.

At the end of the reaction, the solution is preferably centrifuged to separate the larger sized particles therefrom. Some oxide and carbonate will thus be settled. The solution thus prepared will contain between .3 and .8 per cent of lead in colloidal form. The solution may be bottled without special precautions and will remain stable for a number of weeks. The product may be sealed in tubes and heated to 70° C., without affecting its stability. It may also be heated to boiling, which, however, will reduce its stability to only a few days. Deliberate attempt to break down the metallic colloid thus formed required the use of a constant stream of air for two days to completely oxidize one hundred cubic centimeter sample containing .5 per cent lead.

The practice of adding calcium salts to the gelatine, recommended in ordinary directions for the preparation of metallic colloids, is preferably avoided when poly-hy-

droxy compounds are employed as the colloid has a tendency to jell out.

It is understood that the invention is not necessarily confined to the production of lead colloids, as other metallic colloids can be prepared in identical manner, and the invention has a wide application and relates generally to the broad field of metallic colloids. As an example of a particular use of the invention without limiting the invention thereto, the lead metallic colloidal solution prepared finds service as a cancer cure, and the present invention permits a suitable product to be prepared for this purpose.

While the particular process herein described is well adapted to accomplish the objects of the present invention, it is understood the invention includes all such modifications and changes as come within the scope of the appended claims.

I claim:

1. A process of producing a metallic colloid comprising, disintegrating a metal in an aqueous solution of a saccharide and a protective dispersing agent.

2. A process of producing a lead colloid comprising electrically disintegrating lead by forming an arc between lead electrodes submerged in a solution of gelatine, the solution containing glucose.

3. A process of producing a metallic colloid comprising forming an arc between metal electrodes submerged in a solution of protective colloid, the solution also containing a saccharide.

4. A process of producing a metallic colloid for medical purposes comprising, disintegrating a metal in an aqueous solution of gelatin and an aliphatic poly-hydroxy compound capable of retarding oxidation of the metal, said compound having substantially no reducing action.

5. A method of producing a metallic colloid for medical purposes, comprising forming an aqueous solution of gelatin and an aliphatic poly-hydroxy compound capable of retarding oxidation of dispersed metal, electrically disintegrating a metal in said solution while maintaining said solution at a temperature below 30 degrees C., and then removing coarse particles from the colloidal suspension thus formed.

6. A method of producing a metallic colloid for medical purposes, comprising forming an aqueous solution of gelatin and an aliphatic poly-hydroxy compound capable of retarding oxidation of dispersed metal, adjusting the pH of the solution to between 7 and 8, and electrically disintegrating a metal in said solution while maintaining said solution at a temperature below 30 degrees C.

7. A method of producing a lead colloid for medical purposes, comprising forming an aqueous solution of gelatin and an aliphatic poly-hydroxy compound capable of

retarding oxidation of dispersed metal, adjusting the pH of the solution to between 7 and 8, and forming an arc between lead electrodes submerged in said solution while maintaining the solution at a temperature below 5 30 degrees C.

Signed at Santa Barbara, Calif., this 23rd day of September, 1926.

FRITZ E. BISCHOFF.

10

15

20

25

30

35

40

45

50